

(No Model.)

F. V. GREENE.

CONSTRUCTION OF CONCRETE PAVEMENTS.

No. 349,645.

Patented Sept. 21, 1886.

Fig. 1.



Fig. 2.



Witnesses

Edwin T. Jewell,  
W. C. Shaffer

Inventor

Francis V. Greene  
By his Attorney  
Edgarinsbaugh

# UNITED STATES PATENT OFFICE.

FRANCIS V. GREENE, OF NEW YORK, N. Y., ASSIGNOR TO THE BARBER  
ASPHALT PAVING COMPANY, OF WASHINGTON, D. C.

## CONSTRUCTION OF CONCRETE PAVEMENTS.

SPECIFICATION forming part of Letters Patent No. 349,645, dated September 21, 1886.

Application filed March 12, 1886. Serial No. 194,991. (No model.)

*To all whom it may concern:*

Be it known that I, FRANCIS V. GREENE, a citizen of the United States, residing at New York, in the county of New York and State of New York, have invented certain new and useful Improvements in the Construction of Concrete Pavements, of which the following is a specification, reference being had therein to the accompanying drawings.

10 My invention relates to improvements in concrete pavements.

The object of my invention is to prevent the cracking or breaking of concrete pavements incident to thermal changes; and my 15 invention consists in embedding in the body of the pavement wire-netting or similar material which will form a bond and prevent the pavement from separating into seams or cracks.

20 My invention is specially intended to prevent the cracking or breaking of what is commonly known as "asphalt" or other bituminous pavements, but may be applied to other kinds of pavements which are laid in a 25 continuous sheet or unbroken mass.

In asphalt pavements, especially where large areas are to be covered with an unbroken mass or continuous sheet, great difficulty has heretofore been experienced in preventing the separating or cracking of the pavements by the contractions and expansions incident to thermal changes, and in wide 30 streets, and at the crossings of streets the pavements are frequently rendered almost 35 worthless by the thermal changes of one season, examples of which can be seen on the wide avenues and streets of Washington, District of Columbia.

In the drawings, Figure 1 is a top or plan 40 view of a pavement, showing the different layers and the wire-netting. Fig. 2 is a sectional view of the pavement, showing the wire-netting embedded in the wearing course or top layer of the pavement.

45 A indicates the base of the pavement, which is made of hydraulic concrete in the usual manner, and of any desired thickness.

B indicates the top or wearing layer or surface of the pavement, and is composed of asphaltic cement or any other suitable material, but by preference the asphalt cement as laid by Barber Asphalt Paving Company.

50 C indicates the layer of wire-netting which

is embedded in the asphalt top B and serves to hold the same together, and thus prevent 55 the pavement from cracking. The wire-netting which I prefer to use is open mesh, such as is made and used for fences, the wire being galvanized or not, as may be most desirable.

In laying the pavement a portion of the 60 asphalt-cement top is laid on the hydraulic-cement base A in the form of a sticky powder, but not rolled or compressed. The wire-netting is then embedded on the top of this layer of asphalt cement. The balance of the asphalt 65 top is now put down over the wire-netting and heavily rolled so as to thoroughly consolidate and unite this mass of asphaltic cement or concrete with the wire-netting embedded therein. Some little distance below the 70 surface this will effectually prevent the breaking or cracking of the roadway and make a durable and substantial pavement.

As before intimated the wire-netting is intended to be used where large areas are to be 75 covered with an unbroken mass or continuous body of hydraulic or asphalt concrete, so as to prevent the same from being rent or cracked by the contractions and expansions of the pavement incident to thermal changes; but I 80 do not confine myself to such, as it can be used to advantage in all pavements and for foot-walks or drives in parks where concrete pavements are generally affected by the up- 85 heavals of the frost.

I am aware that wire-netting has been used between layers of felt in the manufacture of a roofing fabric, and that emery-wheels made of a plastic material have been strengthened by wire-netting, and such I do not claim.

Having thus described my invention, I claim—

1. A concrete pavement having embedded therein a layer of wire-netting or similar material which will prevent the same from cracking, as set forth.

2. An asphalt concrete pavement or foot-walk having wire-netting embedded in the top layer and some little distance below the wearing surface, as set forth.

In testimony whereof I affix my signature in presence of two witnesses.

FRANCIS V. GREENE.

Witnesses:

ROBERT E. MORRIS.

A. L. BARBER,